

Feb. 11, 1930.

H. DEBAUCHE

1,746,767

METHOD OF PRODUCING FUEL FOR INDUSTRIAL AND DOMESTIC PURPOSES

Filed July 6, 1927

3 Sheets-Sheet 1



By: Monroe & Clark  
Atys.

Feb. 11, 1930.

H. DEBAUCHE

1,746,767

METHOD OF PRODUCING FUEL FOR INDUSTRIAL AND DOMESTIC PURPOSES

Filed July 6, 1927

3 Sheets-Sheet 2



Fig. 2.



Fig. 4.

H. Debauche  
Inventor

By: Marks & Clarke  
Attest.

Feb. 11, 1930.

H. DEBAUCHE

1,746,767

METHOD OF PRODUCING FUEL FOR INDUSTRIAL AND DOMESTIC PURPOSES

Filed July 6, 1927

3 Sheets-Sheet 3



H. Debauche  
INVENTOR

by: Marks & Clark  
A.T.S.

## UNITED STATES PATENT OFFICE

HUBERT DEBAUCHE, OF NEAR CHARLEROY, BELGIUM

## METHOD OF PRODUCING FUEL FOR INDUSTRIAL AND DOMESTIC PURPOSES

Application filed July 6, 1927, Serial No. 203,860, and in Great Britain November 29, 1926.

This invention relates to the commercial utilization of lignite, cannel coal and similar carbonaceous matter so that it may be transformed into a fuel of high calorific value.

5 It has been suggested before reducing coal to a finely divided condition for combustion in furnaces, to subject the coal to low temperature distillation to remove the tar and tar oil content so as to obtain a fragile residue having a volatile content of about 6% to 18%. On the discharge of this residue from the retort it is quenched with water or steam and reduced to powder.

The present invention relates more particularly, however, to a process described in the specification of prior British Patent No. 254,964 which comprises the subjecting of lignite or the like to low temperature distillation, after which the material whilst retaining a sufficiency of heat is successively screened, graded, mixed and finally agglomerated to form briquettes. As described in such specification the operations were uninterruptedly and continuously maintained and 25 any intermediate reheating avoided.

As a result of observation and experiment now made by the inventor, it has appeared that it is possible to so control the method and apparatus that various distinct grades 30 of semi-coke may be produced to serve as:

(a) Direct fuel for domestic grates;  
(b) Direct fuel for furnaces for industrial purposes, and  
(c) Material graded to any desired size 35 under 5 m/m intended (1) to be agglomerated and made into briquettes of coarse or fine grain as desired, or (2) to be directly used in furnaces constructed for burning pulverized coal.

40 This production and grading of semi-coke is facilitated by the kind of retort or coke oven chosen in which the raw material is first treated or distilled. For example:

45 (1) If a low temperature distillation oven is selected in which the fuel is motionless during the distilling operation or else only moves slowly without being energetically disturbed, then if a non-caking fuel is introduced in 50 fragments as large as 40 m/m in size, semi-

coke is obtained the fragments of which measure up to 35 m/m.

(2) When a low temperature distillation oven is chosen in which is placed a non-caking fuel not exceeding 10 to 12 m/m in size, 55 and it is moved about energetically during the whole of the distilling operation, then the largest fragments of semi-coke obtained rarely exceed 8 m/m in size.

If the fuel is pulverized before being introduced into the retort, then the resulting product will be pulverulent semi-coke.

The object of the present invention is such a treatment of lignite, cannel coal or similar carbonaceous material that after a primary 65 grading of the semi-coke into two definite sizes the larger grade is used directly and the smaller grade is subjected to a second selective grading from which briquettes or ovoids of a finer or coarser grain may be prepared at choice or a grade obtained that may be directly used in furnaces for burning pulverized fuel.

The invention consists in an improved method for the transformation of lignite, 75 cannel coal or similar carbonaceous material into fuels of high calorific value, consisting in subjecting the raw material to low temperature distillation, cooling the semi-coke as it issues from the retort or oven screening it 80 so as to obtain a primary grading whereby the aggregate is separated into pieces above and below 5 m/m respectively, the former being led away for use as a direct fuel that may be further graded if desired, and the latter 85 being led away for a secondary grading so as to produce semi-coke from 0 to 1/6 m/m, or 0 to 1/4 m/m to be pulverized and used directly in furnaces constructed to burn pulverized fuel or to produce one or more of a 90 number of grades from 0 m/m to 1/6 m/m, 0 to 1/4 m/m, 0 to 1/3 m/m, 0 to 1/2 m/m, 0 m/m to 1, 2, 3, 4 or 5 m/m respectively, and subsequently agglomerating a selected second- 95 ary grade or grades as desired to form briquettes or ovoids, which may be if necessary subjected to further distillation, the above operations being executed progressively, continuously or non-continuously as desired in 100

a determined sequence for each particular product desired.

The invention also consists in apparatus for realizing in practice the above-stated method of treating low grade fuels.

Referring now to the accompanying drawings:—

Figure 1 is a diagrammatic view in elevation of one form of apparatus.

Figure 2 is a similar view to Figure 1 of part of the apparatus according to a modified construction.

Figure 3 is a plan view of Figure 1, and Figure 4 is a plan view of Figure 2.

In carrying the invention into effect more especially with reference to Figures 1 and 3, *a* indicates one or more vertical retorts or ovens into which the lignite, cannel coal or the like is fed at the top. These apparatus or ovens are only indicated by way of example because ovens and apparatus of other systems may also be used. Figure 3 illustrates by way of example, a battery of six of such retorts and *a'* indicates the means by which the desired proportion of volatile constituents is led away from the base of each retort to the usual plant *a*<sup>2</sup> for the recovery of the tar, benzols, gas and the like. As the details of this apparatus are well known and do not form part of the present invention, it is not further described. At the bottom of each retort is an outlet *b* for the semi-coke produced.

It has been observed by the inventor that certain semi-cokes obtained from low temperature distillation ignite spontaneously upon contact with the air, that is upon removal from the retort, and means are therefore provided to cool the semi-coke, but the extent of such cooling is however variable according to the use which is to be made of the semi-coke. Thus where the product will be subsequently agglomerated the semi-coke will be cooled down to about 180° C. so that there will be no necessity for any intermediary re-heating to facilitate its manufacture into briquettes or ovoids, but if the semi-coke is to be stored it is cooled down to about 40° C.

For this purpose as the semi-coke leaves the outlet *b* it is received in a chamber *c* closed off from the atmosphere and cooled by a water circulating system of which *d* is the inlet pipe and *e* the outlet. This cooling chamber is particularly described in the specification of British Application No. 18159 of 20th July 1926. The fuel upon leaving the chamber *c* is received by a closed-in screen *g* of any usual construction where a primary separation is effected into two grades, viz, pieces above 5 m/m in size that remain on the sieve, and pieces under 5 m/m that pass through. The larger grade passes by way of a chute *h* down to a conveyor *k* by which it is carried away to a storage, each

retort having its own chute, and all the chutes serving the conveyor *k*. Both the conveyor and the chutes are closed in by suitable means so as to prevent the diffusion of dust in atmosphere which might thereby cause an explosion, and if desired, these enclosed spaces may be filled with an inert gas.

It is to be noted that this primary separation of the fuel takes place as close as possible to the cooling chamber *c* as it is of advantage that at least the larger grade of 5 m/m and upwards shall not receive any unnecessary handling owing to its friable nature. This separated larger grade is intended for direct burning as in domestic fire-grates, and furnaces of steam boilers and to suit it to these respective purposes it may for instance be subjected to further screening at the end of the conveyor *k* to obtain (firstly) an aggregate of a size from 5 to 8 m/m adapted to be burned in the furnaces of steam boilers and (secondly) an aggregate of 8 m/m and above suitable for domestic fire-grates.

The aggregate which passes through the screen *g* of a size from 0 to 5 m/m to be subsequently pulverized or agglomerated is led down a closed chute *l* from each retort, and all discharge into a conveyor *m* from whence by means of a duct *n* it passes into the lower end of a completely closed conveyor *o* by which the aggregate is raised and transferred to a duct *p* which delivers it either into a pit *q* or onto a screen *r*. In a case where the aggregate coming from the retort is in a pulverulent condition, the screen *r* is moved so that it falls direct into the pit *q*, from whence it is taken by the conveyor *u* to the agglomerating plant or by another conveyor which directs it to a furnace constructed for burning pulverized coal, but when the aggregate is of a size between 1 and 5 m/m inclusive the screen *r* is moved into the path of the falling aggregate and caught.

When making agglomerate from semi-coke of 0 m/m to 5 m/m the semi-coke coming through the conveyor *o* is carried to the duct *p* which delivers it directly to the pit *q* without it passing through the screen *r*.

The screen *r* is used to determine the granular structure of the briquettes or ovoids that are to be produced, whether it is to be fine or coarse. For instance if the grains are not to exceed 2 m/m in size, then a screen *r* is placed in position to catch the aggregate up to 5 m/m.

All the grains below 2 m/m will pass through the screen and fall into the pit *q*, but the grains above this size pass along the screen and are led away to a crusher *s* and after being treated therein it falls into a pit *t*, from whence it is raised by a conveyor *j* and is returned to the conveyor *o* to again pass the screen *r* the aggregate being now of the requisite size and being delivered to the pit *q*. Thus by changing the screen to the size

required, so the aggregate delivered to the pit  $q$  will be of the corresponding size, and whilst that particular screen is in position, the pit will receive that size only.

5 For a simplification of the plant, a modification may be used as indicated in Figures 2 and 4, according to which the screen  $g$  below each oven or retort is omitted, and replaced by a single screen  $g'$  placed immediately in 10 front of the screen  $r$ . All of the semi-coke produced by the oven and coming from the chamber  $c$  falls into a duct  $l$ , the series of which all lead the semi-coke to the conveyor  $m$  from whence by means of the duct  $n$  it 15 passes into the lower end of a completely closed conveyor  $o$  by which the aggregate is raised and transferred to the screen  $g'$  of any usual construction where a primary separation is effected into two grades, viz., pieces 20 above 5 m/m in size that remain on the sieve, and those under 5 m/m that pass through.

The larger grade is passed on to the conveyor  $k$  by which it is carried away to storage. The aggregate however which passes 25 through the screen  $g'$  of a size from 0 to 5 m/m to be subsequently agglomerated or pulverized by the crusher  $s$  for use in furnaces specially intended to burn the pulverized fuel, passes on the screen  $r$  which is arranged as above described.

When it is desired to produce a compressed and agglomerated fuel possessing exceptionally high cohesion and having very feeble permeability to water, it is necessary to crush 35 the semi-coke very fine and therefore in this case a screen  $r$  would be employed having a mesh narrower than 1 m/m.

When however the semi-coke is to be pulverized so that it may be burned in furnaces 40 adapted to burn pulverized fuel, it will be necessary to select a very fine screen  $r$  capable of producing semi-coke of 0 to 1/6 m/m and 0 to 1/4 m/m which will be pulverized at the place where it is to be used by any well-known apparatus, the semi-coke refuse being 45 always directed toward the crusher  $s$  and the product from said crusher being returned to the screen  $r$ ; the fuel that has however passed through the sieve will not be conducted towards the agglomerating plant but will fall 50 into the pit  $q$  from whence it is taken by a chain or other conveyor which will deliver it to wagons or magazine hoppers or to where it is to be directly used.

55 It is possible to replace the screen  $r$  and the crusher  $s$  mentioned above by a crusher adapted to supply a semi-coke crushed to the size required.

Returning to Figures 1 and 3, from the 60 pit  $q$ , the aggregate of the size chosen is raised by another completely closed conveyor  $u$  and fed to one of two conveyors  $w, x$ , which supply it to one of two towers  $y, z$ , respectively. Which of these conveyors and towers 65 are used depends upon the position of a flap

valve 10, but under normal conditions the aggregate will be delivered to the conveyor  $w$  and the smaller of the two towers  $z$  on its way to be agglomerated.

Should there be however a stoppage in the agglomerating part of the plant, the valve 10 70 is adjusted into its alternative position to deflect the aggregate to the conveyor  $w$  and thence into the tower  $y$ , this being of larger capacity intended to act for storage. With 75 the regular operation of the plant the small capacity of the tower  $z$  is sufficient so as to avoid any accumulation which is undesirable in view of the temperature of the aggregate and that no cooling is desirable at that stage of the process. Owing, however, to the greater capacity of the tower  $y$  and the accumulation of heated aggregate that will take 80 place therein when and if it is used, it is to be understood that the semi-coke will be cooled down to 40° C. in the chamber  $c$  of each of the retorts or ovens, this being effected by increasing the flow of cooling water by means of a valve fitted in the pipes  $d$  or  $e$  or both.

The lower ends of the towers  $y, z$ , converge 85 at one outlet 11 where a suitable measuring device 12 permits definite charges of aggregate, or controls the discharge thereof during a given time, into one end of a conveyor 13. Alongside of the tower  $y, z$  is arranged another tower 14 which contains a pulverized 90 binder such as pitch which is supplied from a crusher 15 and fed from thence to the tower 14 by conveyors 16, 17. The discharge of pitch is controlled by a measuring device 18 whence it passes into the other end of the conveyor 13. The two measuring devices 12 and 18 deliver to the conveyor 13 the proportionate quantities of aggregate and pitch 95 and these are mixed together and discharged from the conveyor by the fact that it is a worm conveyor, the threads of which at each end are respectively right and left hand. The action of the worm therefore draws the aggregate and pitch towards one another so 100 that they are discharged together at the common outlet 19 from whence they pass in a mixed condition to a conveyor 20 in which their mixing is finished and are led away to be briquetted. In the example shown, the 105 towers  $y, z$  and 14 are duplicated and two conveyors 20 are used for leading away the mixed aggregate, thus one of the conveyors 20 passes it by way of a mixer 21 to a briquetting press 22 from which the finished briquettes pass by the conveyor 23, and the other conveyor 20 forwards the mixed aggregate 110 by way of mixer 24 to an ovoid making press 25. From this latter press the ovoids are delivered to a storage 26, or if desirable they 115 are passed by way of a chute 27 to a retort or oven 28 to distil off any excess of volatile content, so that it may be recovered. The fuel thus treated may be considered as smokeless burning fuel having very high cohesion 120

125

130

and calorific value so that it is comparable to the best anthracite for use in domestic fire-grates.

By the foregoing arrangement it will be understood that depending upon the kind of screen *r* selected, so the semi-coke may be pulverized as desired and briquettes or ovoids may be made of an aggregate formed of pieces ranging from 0 to 1, 2, 3, 4 or 5 m/m respectively and varying in granular structure from fine to coarse.

It has been observed in the course of experiments that with an industrial low temperature distilling retort of class No. 1 (where the fuel is substantially motionless) when there was placed in an oven in 8 consecutive days approximately 100 tons of lignite containing 20% of water and the fragments of which varied from 0 m/m to 35 m/m, there was produced a semi-coke containing: firstly, approximately 45% of fuel of a size varying from 5 to 30 m/m (of which 2/3rds was of a size from 5 to 8 m/m whilst the remaining 1/3rd was of a size between 8 to 30 m/m); secondly, approximately 55% of fuel from 0 m/m to 5 m/m.

On the other hand with a retort of the second class in which the fuel was freely agitated, there was a yield of semi-coke containing: firstly, an aggregate of 20% of a size varying from 5 to 8 m/m; secondly, approximately 80% of any size varying from 0 to 5 m/m.

The semi-cokes produced by these various distilling ovens or retorts are characterized by being completely deprived of moisture; they usually contain 8 to 12% of volatile substances but this can nevertheless be reduced to only 3 to 4% of volatiles, where it is desired to manufacture an agglomerate comparable with anthracite.

In spite of the small volatile content, they burn admirably and give out an extreme heat, with absolutely no smoke, very easy ignition and for an ash content of 6% their calorific value exceeds 8,000 calories, per kilogramme.

These semi-cokes therefore form a fuel of the first order and they must be used when possible in the state in which they are produced, that is to say, without any further preparation.

It has been observed that the fragments of semi-coke the dimensions of which vary from 5 to 8 m/m, burn perfectly in the furnaces of steam boilers, upon grates the bars of which are spaced about 4 1/2 m/m apart approximately and that an aggregate that exceeds in size 8 m/m and up to 30 m/m can be successfully used in domestic fire-grates.

Also in the course of experiments, there have been manufactured 5 grades of compressed fuel of a size from 0 m/m to 1 m/m—0 m/m to 2 m/m—3 m/m—4 m/m—5 m/m. During combustion the five different agglomerates have given the same calorific value,

but the agglomerate manufactured with semi-coke of a size from 0 m/m to 1 m/m gave maximum cohesion and density for a minimum capacity for absorbing moisture whilst requiring more pitch.

On the contrary, the agglomerate manufactured with semi-coke 0 m/m to 5 m/m, gave the minimum cohesion and density with a maximum capacity for absorbing moisture whilst requiring less pitch.

It can be concluded that the finest semi-coke will give the hardest agglomerate, the most dense and the least pervious to water, whilst the semi-coke of larger size will give a compressed fuel which is the least hard, the least dense and the most pervious to water.

It has been found that after testing the cohesion of the agglomerate obtained with semi-coke of 0 to 5 m/m in size was 25% less than that of the agglomerate obtained with the semi-coke of fragments 0 m/m to 1 m/m whilst the difference between their densities was 6%.

After a complete immersion in water for 30 consecutive hours, the agglomerate obtained with the semi-coke of fragments 0 to 5 m/m absorbed 4 1/2 times more water than the agglomerate obtained with the finest, that is 0 to 1 m/m.

As regards the quantity of pitch employed for the agglomerate of 0 to 5 m/m, it was less than for the aggregate of 0 to 1 m/m by about 7.50%.

With the intermediate fuels, that is to say 0 to 2 m/m, 0 to 3 m/m and 0 to 4 m/m, the differences were practically proportional.

It is evident also that with a semi-coke of which the coarser size is below 1 m/m (1/6, 1/4 m/m—1/3rd m/m, 1/2 m/m or otherwise) it is possible to obtain more cohesion and density than with 0 m/m to 1 m/m.

In conclusion, the foregoing description discloses a system and apparatus for the transformation of fuel which is usually regarded as of low grade value into fuels of high value which system may be carried on continuously or non-continuously.

There is no danger of fire from the use of the apparatus, and the apparatus may be constructed so as to form an unbroken system of operations or so constructed that the operations may be intermittent or continuous as desired.

Having now described my invention, what I claim as new and desire to secure by Letters Patent is:—

1. A method for the transformation of a solid distillable carbonaceous material of low calorific value into fuels of high calorific value, consisting in subjecting the said material to low temperature distillation and continuously separating the volatile constituents from the solid portions, cooling the solid portion to below 180° C. as it issues from the re-

tort and before it is exposed to air, screening the solid portion while still warm whereby the aggregate is separated into pieces above and below 5 m/m respectively, the former constituting a fuel capable of further grading, subjecting the latter to a selective secondary screening, and dividing the selected screenings obtained to be agglomerated while still warm to form briquettes, in one case, and to be led away so as to be used for making a pulverized fuel in the other case.

2. A method as claimed in claim 1, in which the oversize screened material from the selective secondary screening while still warm is submitted to crushing and the crushed product returned to the selective secondary screening operation.

3. A method as claimed in claim 1 in which the agglomerated material is mixed with pitch and formed into briquettes.

In testimony whereof I have signed my name to this specification.

HUBERT DEBAUCHE.

25

30

35

40

45

50

55

60